

## UNITED STATES PATENT OFFICE

FOORD VON BICHOWSKY, OF GLENDALE, CALIFORNIA, ASSIGNOR TO TITANIA CORPORATION, OF LOS ANGELES, CALIFORNIA, A CORPORATION OF CALIFORNIA

## METHOD FOR PRODUCING TITANIUM COMPOUNDS

No. Drawing.

Application filed May 22, 1929. Serial No. 365,233.

The present invention relates especially to stabilizing the interaction of titanium nitrogen compounds and nitric acid with the object of obtaining new and also more uniform products.

In my United States Letters Patent Number 1,742,674, dated January 7, 1930, there is described a method for producing titanium oxide from titanium nitrogen compounds by 10 acting upon them with nitric acid either alone or in the presence of sulphuric acid whereby only about a third of the nitrogen of the titanium nitrogen compound is recoverable in the form of an ammonium compound the remainder escaping presumably in 15 the form of nitrogen gas. The following equation illustrates that reaction:



20 Further I said in my copending application for Letters Patent Serial Number 320,762, filed November 20, 1928, that most of the nitrogen of the titanium nitrogen compound 25 pounds is lost when one acts upon them with nitric acid in the presence of sulphuric acid. In this instance the object of the invention was the formation of new types of acid 30 titanium sulphates.

It is, therefore, easy to see that if some or even more of the combined nitrogen of the titanium nitrogen compound, and by 35 titanium nitrogen compound I mean titanium nitride or titanium cyanonitride and especially the reactive nitrogen compound 40 prepared by the methods of my United States Letters Patent 1,408,661, dated March 7, 1922, could be recovered in a combined and marketable form, say as ammonia or a salt 45 thereof, that such a by-product would prove to be quite an asset to the above mentioned processes. In addition to ammonium compounds there is also the possibility of recovering some of the combined nitrogen in the 50 form of oxides of nitrogen. The following equation will show one case where this might happen:



55 There is of course the possibility that other

reactions might take place or that both reactions, shown by the equations could occur simultaneously.

Such considerations led me to study means for controlling or slowing down the reactions in such a way that a maximum yield of 55 nitrogen compounds might be formed together with a minimum amount of free nitrogen. As a result of those studies I have now discovered that if substances, be added to the 60 reactants, capable of giving in solution ions of phosphorus compounds that these ions act as inhibitors or negative catalysts and cause the nitric acid and titanium nitrogen compound to interact more slowly. Among the 65 substances suitable for this purpose I mention soluble phosphates or phosphoric acid or even phosphites or such compounds as can be oxidized by nitric acid to give phosphates. One may also use compounds such as calcium 70 phosphate which under the action of sulphuric or other acids can form soluble phosphates.

If, therefore, nitric acid or a suitable nitrate be allowed to interact with a titanium 75 nitrogen compound, or compounds, in the presence of water and sulphuric acid or a halogen acid or mixtures of such acids and there be added to these reactants a small amount of a substance capable of yielding a 80 phosphate ion a smooth reaction takes place giving as by-products a uniform yield of nitrogen compounds. This reaction therefore gives ammonium compounds, often associated with free nitrogen and nitrogen oxides, 85 together with an excellent yield of a semi-colloidal partly hydrated titanium oxide of a white or bluish-white color having good covering power and possessing a specific gravity lower than that of any known titanium 90 dioxide.

As an example of the carrying out of my discovery, as applied to the production of titanium oxide, I will give the following experiment but it is to be understood that I do 95 not confine the scope of my invention to this example as one skilled in the art may readily vary the details.

40 grams of concentrated sulphuric acid were poured into 40 cubic cms., of cold water 100

and when the diluted acid was cool it was poured over 35 grams of commercial titanium cyanonitride contained in a 1500 cubic centimeter beaker. Next 35 grams of commercial sodium nitrate (chile saltpeter) were dissolved in 60 cubic cms., of water and to this solution were added 3 grams of sodium phosphate. The aqueous solution of sodium nitrate and sodium phosphate was now poured into the large beaker containing the sulphuric acid-titanium cyanonitride mixture. The materials were stirred constantly and if necessary to start or accelerate the reaction they were warmed on the water bath. The reaction went smoothly and after 24 hours no more reddish colored cyanonitride was discernable and no more gas was given off. Then the white titanium oxide paste was greatly diluted with water allowed to settle and the excess water, which contained ammonium sulphate and sodium sulphate, was siphoned off. This washing by settling and decantation was continued until the wash water was free of iron and only faintly acid. The dioxide of titanium so obtained was so finely divided that it passed through filter paper. In order to remove the last traces of acid remaining in the titanium oxide paste it was neutralized with ammonia. It is evident that in place of using ammonia for this neutralization that one could use other bases such as lime or barium hydrate or even faintly basic or neutral substances such as barium carbonate or the chlorides of barium or calcium or such other compounds as would give volatile acids upon drying.

After the pasty titanium oxide had been thus neutralized with ammonia more water was added. Next a few cubic centimeters of dilute hydrochloric acid were poured in. This acid was added to facilitate the further washing of the oxide as the almost colloidal titanium dioxide settles out more rapidly from solutions containing halogen ions or having a definite hydrogen ion concentration. After one or two washings to remove any ammonium sulphate or other undesired substance the settled out hydrated titanium dioxide was evaporated to dryness.

There was thus obtained a white to bluish white hydrated titanium oxide containing, when dried at just below 100° cent., about 8% by weight of water. The dry powder had a specific gravity of 2.72.

Such an oxide makes, when worked up in a suitable vehicle, an excellent pigment and because of its low specific gravity it does not settle out easily from liquid paints. The oxide may be completely dehydrated by heating to below a red heat and one thus obtains a material usually not quite as white but useful for compounding with rubber or linoleum or for any other purpose for which titanium oxide is ordinarily used.

The working up of the wash water for am-

monium compounds and the recovery of nitrogen oxides from the gases given off during the reaction follows well known practices.

It is obvious that when using different combinations of reactants that different temperatures, pressures or concentrations may have to be employed to obtain the desired results but these changes are well within the scope of studies made by one skilled in the art. I do not confine myself to such variations or to the example as given but only to the claims.

What I claim as my invention is:

1. Method for producing titanium compounds which consists in stabilizing the interaction of nitric acid and titanium nitrogen compounds by carrying out the reaction in the presence of a phosphate ion. 70

2. Method for producing titanium compounds including titanium oxide of low specific gravity which consists in stabilizing the interaction of nitric acid and titanium nitrogen compounds in the presence of water by employing phosphoric acid as an inhibitor. 85

3. Method for producing titanium compounds including titanium oxide of low specific gravity which consists in stabilizing the interaction of nitric acid and titanium nitrogen compounds in the presence of water and sulphuric acid by employing alkali metal phosphate as an inhibitor. 90

4. Method for producing titanium compounds including titanium oxide of low specific gravity which consists in stabilizing the interaction of nitric acid which is generated in situ by sulphuric acid acting upon sodium nitrate and titanium nitrogen compounds while in the presence of water and sulphuric acid by employing alkali metal phosphate as an inhibitor. 100

5. Method for producing titanium compounds including titanium oxide of low specific gravity which consists in stabilizing the interaction of nitric acid which is generated in situ by sulphuric acid acting upon an alkali metal nitrate and titanium nitrogen compounds while in the presence of water and sulphuric acid by employing alkali metal phosphate as an inhibitor. 110

6. Method for producing titanium compounds including titanium oxide of low specific gravity which consists in stabilizing the interaction of nitric acid and titanium nitrogen compounds in the presence of sulphuric acid and water by employing calcium phosphate as an inhibitor. 115

7. Method for producing titanium oxide of low specific gravity which consists in stabilizing the interaction of nitric acid and titanium nitrogen compounds in the presence of sulphuric acid and water by employing a soluble phosphate as an inhibitor and recovering semi-colloidal titanium oxide having a specific gravity less than 2.9. 125

FOORD VON BICHOWSKY. 130